

## UNITED STATES PATENT OFFICE

DAVID RONALD TULLIS, OF SUTTON COLDFIELD, AND PERCY OAKLEY, OF LIVERPOOL,  
ENGLAND

## PRODUCTION OF AN ALUMINIUM ALLOY

No Drawing. Application filed September 8, 1932, Serial No. 632,184, and in Great Britain October 27, 1931.

This invention relates to the production of a refined aluminium alloy having stain-

less properties as well as hardness. the remainder being substantially alumin-

The improved alloy contains, besides 5 aluminium, magnesium, chromium, manganese and titanium, and may also contain a small quantity of boron, as well as iron and silicon.

In testimony whereof we have signed our names to this specification.

D. R. TULLIS. 50  
PERCY OAKLEY.

In the production of the improved alloy 10 a quantity of chromium-aluminium alloy rich in chromium is added to a bath of already molten aluminium, the heating being continued so that the molten condition is maintained. There is then added to the 15 bath manganese-titanium-aluminium alloy rich in manganese and titanium. Then elemental magnesium is added, the molten condition being maintained.

55

The vapour of boron trichloride or the 20 volatile halide of a metal having a grain-refining influence may then be introduced into the bath as described for example in the specification of U. S. Letters Patent No. 1,636,881 issued 26th July, 1927.

60

25 By way of example suitable proportions of the ingredients of the alloy are as follows:—

Percent

|           |       |         |
|-----------|-------|---------|
| Chromium  | ..... | .1 to 1 |
| Manganese | ..... | .2 to 2 |
| Titanium  | ..... | .1 to 1 |
| Magnesium | ..... | .5 to 5 |

70

the remainder being aluminium, and, in certain cases, small quantities of boron or other 35 element introduced by the refining operation.

75

Iron and silicon are usually present as impurities in the aluminium, up to .75% of iron and .75% of silicon.

80

We claim:—

40 A refined aluminium alloy consisting of:—

Percent

|           |       |         |
|-----------|-------|---------|
| Chromium  | ..... | .1 to 1 |
| Manganese | ..... | .2 to 2 |
| Titanium  | ..... | .1 to 1 |
| Magnesium | ..... | .5 to 5 |

85

90